

## UNITED STATES PATENT OFFICE

DALE M. PHILLIPPI, OF DAYTON, OHIO, ASSIGNOR TO THE KAY &amp; ESS CO., OF DAYTON, OHIO, A CORPORATION OF OHIO

## ENAMEL IMITATION LEATHER FINISH

No Drawing.

Application filed July 22, 1929. Serial No. 380,246.

This invention relates to enamels and varnishes, and particularly to a finish that imitates the appearance of leather.

It is the object of this invention to provide an enamel varnish which, when applied to a suitable surface, will give to it a finish imitating leather.

It is a further object of this invention to eliminate all blown oils and preoxidized oil thereby materially reducing the cost and improving the product.

It is an additional object to provide an enamel varnish which will employ in the formula cheaper gums and resins than heretofore have been possible in connection with varnishes of this type.

A typical formula is the following:

|                         | Pounds     |
|-------------------------|------------|
| Amberol B/S 1 Lt.       | 67         |
| Litharge                | 3½         |
| Manganese linoleate     | 8½ (solid) |
| Cobalt linoleate        | 2 (solid)  |
|                         | Gallons    |
| China wood oil          | 20         |
| Linseed oil             | 2½         |
| Heavy petroleum naphtha | 14         |
| Light petroleum naphtha | 14         |

A suitable substance to be used as Amberol, in the above formula, is disclosed in U. S. Letters Patent No. 1,623,901, dated April 5, 1927.

In order to prepare this varnish, I first take 20 gallons of China wood oil and 2½ gallons refined linseed oil. These oils are mixed and heated at a normal rate to 480° F. They are then pulled from the fire. These oils may undergo an automatic rise in temperature thereafter beyond 480° F., but this is unnecessary and too great a rise should be avoided.

When the temperature of these oils has started to drop reaching approximately 475° F., I add 3½ pounds of litharge stirring until the litharge is taken up by the oil. The temperature of this batch is then run back and forth between 460° and 470° F. being held within this range for approximately 30 minutes and in some cases a little longer until

sufficient body has been imparted to the oil and litharge.

Thereafter I add 8½ pounds of manganese solid linoleate and 2 pounds of cobalt solid linoleate. These soluble driers melt into the batch.

I then add 67 pounds of synthetic resin solid, known to the trade as "Amberol B/S 1 Light." This is melted at a low heat. Then the temperature is carried back to approximately 425° F.

I then reduce the batch at once with 14 gallons each of heavy and light petroleum naphtha.

The resulting compound may be used by itself or in combination with the product of the formula hereinafter recited. If used with the next formula, they can be mixed together in proportion as high as one part each.

This formula is as follows:

|                         | Pounds  |
|-------------------------|---------|
| South Sea gum           | 67      |
| Litharge                | 3½      |
| Manganese linoleate     | 8½      |
| Cobalt linoleate        | 2       |
|                         | Gallons |
| China wood oil          | 20      |
| Linseed oil             | 2½      |
| Heavy petroleum naphtha | 20      |
| Light petroleum naphtha | 20      |

The cooking is carried out in this manner.

Sixty-seven pounds of South Sea gum are run in the ordinary approved fashion customary in varnish making. Then 20 gallons of China wood oil and 2½ gallons of refined linseed oil are mixed and heated slowly until they reach 300° or 350° F., then they are added slowly to the gum when the latter has been well run.

The mixture is then carried to a temperature of 460° to 470° F. and held within this range in order to impart body to the mixture for about 30 minutes or a little longer.

I then stir into the batch 3½ pounds of litharge until it is taken up and fully incorporated in the batch. The 8½ pounds of manganese solid linoleate and 2 pounds of

cobalt solid linoleate are allowed to melt in the batch.

I then reduce at once with 20 gallons each of heavy and light petroleum naphtha.

5 Turpentine may be substituted for the naphtha. Either the natural gum or a synthetic product as Amberol may be employed. When the natural product is used the result is a liquid of greater viscosity.

10 The fundamental basis is the combination of a gum and a low cooked China wood oil. The litharge has the function of drying the compound through and through while the manganese and cobalt linoleates act primarily as surface or finish driers. The naphthas act as thinners. The linseed oil is an anti-polymerizing agent.

15 Be it understood that the result of my invention is applied to any suitable surface and 20 baked in the usual manner which brings about the appearance of leather on the surface so treated with my product.

25 It will be understood that I desire to comprehend within my invention and within the scope of my claims such modifications as may be fairly comprehended within such claims and invention due to the necessary modifications to adapt my invention to varying conditions of supply and of use and to varying 30 purposes.

Having thus fully described my invention, what I claim as new and desire to secure by Letters Patent is:

35 1. In a method of manufacturing and improving varnish or enamel for imitating leather finishes mixing China wood oil and linseed oil, heating said oils to approximately 480° F., cooling the oil, incorporating litharge therewith, holding the temperature between 40 approximately 460° to 470° F., for approximately 30 minutes, adding manganese linoleate and cobalt linoleate, and adding a synthetic resin, restoring the temperature to approximately 425° F.

45 2. In an improved method of producing an imitation leather finish in a varnish, mixing 20 gallons of China wood oil and 2 1/4 gallons linseed oil, heating to 480° F., allowing to cool to approximately 475° F., adding 3 1/2 50 pounds litharge, holding the temperature between 460-470° F. for approximately 30 minutes, adding 8 1/2 pounds manganese linoleate and 2 pounds cobalt linoleate, adding 67 pounds of synthetic resin restoring the temperature to approximately 425° F. and reducing the batch with 14 gallons each of heavy and light petroleum naphtha.

In testimony whereof I affix my signature.  
DALE M. PHILLIPPI.